

# United States Patent [19]

Levanon et al.

[11] Patent Number: 5,012,300

[45] Date of Patent: Apr. 30, 1991

[54] TWO-COLOR IMAGING SYSTEM AND PROCESS

[75] Inventors: Moshe Levanon; Israel Grossinger; Yossi Adam, all of Rehovot, Israel; Benzion Landa, Edmonton, Canada

[73] Assignee: Spectrum Sciences B.V., Rotterdam, Netherlands

[21] Appl. No.: 268,855

[22] Filed: Nov. 8, 1988

Related U.S. Application Data

[63] Continuation-in-part of Ser. No. 202,569, Jun. 6, 1988, abandoned.

[51] Int. Cl.<sup>5</sup> G03G 15/01; G03G 15/10

[52] U.S. Cl. 355/328; 355/257; 355/77; 430/32

[58] Field of Search 355/257, 328, 77; 430/32

[56] References Cited

U.S. PATENT DOCUMENTS

- 3,381,662 5/1968 Kolb .  
3,793,205 2/1974 Metcalfe .  
4,023,968 5/1977 Amidon et al. .... 355/257 X  
4,045,219 8/1977 Bean ..... 355/328 X  
4,068,938 1/1978 Robertson .  
4,111,151 9/1978 Ruckdeschel .  
4,250,239 2/1981 Sakai et al. .... 430/42  
4,264,185 4/1981 Ohta .

- 4,310,238 1/1982 Mochizuki et al. .... 355/12  
4,411,976 10/1983 Landa et al. .  
4,562,129 12/1985 Tanaka et al. .  
4,731,634 3/1988 Stark ..... 355/328  
4,830,945 5/1989 Wong .  
4,860,924 8/1989 Simms et al. .... 222/56  
4,877,698 10/1989 Watson et al. .... 430/45

FOREIGN PATENT DOCUMENTS

- 53-121623 12/1978 Japan .  
55-124156 9/1980 Japan .  
59-116764 11/1984 Japan .  
61-223853 10/1986 Japan .  
61-189563 1/1987 Japan .  
1322385 7/1973 United Kingdom .

OTHER PUBLICATIONS

JP 62-144184, 12/87, Japan.

Primary Examiner—R. L. Moses  
Attorney, Agent, or Firm—Sandler, Greenblum & Bernstein

[57] ABSTRACT

Dual color imaging process and system providing formation of an image having adjacent first and second areas respectively containing first and second types of pigmented particles undesirably separated by third areas relatively free of particles of the first and second types and causing the image to flow into the third areas, thereby at least partially eliminating the third areas.

50 Claims, 6 Drawing Sheets





FIG. 1



FIG. 2A



FIG. 2B



FIG. 2C



FIG. 2D



FIG. 3



FIG. 4



FIG. 5

FIG. 6

## TWO-COLOR IMAGING SYSTEM AND PROCESS

## REFERENCE TO RELATED APPLICATION

This is a continuation in part of U.S. Pat. Application Ser. No. 202,569. PROCESS FOR OBTAINING VISUALLY COLORED COPIES ON A SUBSTRATE, filed 6 June, 1988 now abandoned.

## FIELD OF THE INVENTION

The present invention relates to dual color imaging.

## BACKGROUND OF THE INVENTION

In color imaging systems, it is known to print two or more superimposed colors on a substrate by separate operations. Printing in two colors is useful, for example, when it is desired to highlight particular sections of documents such as in accounts, where material may be typewritten in two colors, in stationery with two printed colors and so forth. Printing (or copying) in two or more colors generally requires a process which incorporates two passes as well as accurate registration of the two or more superimposed colors.

In U.S. Pat. No. 4,068,938 (Robertson), there is described a process in which a two color plus background copy is obtained from a two color plus background original. According to Robertson's concept, the pairs of colors are chosen according to the response characteristics of the photoconductive surface on which the electrostatic latent image is formed. Thus the electrostatic latent image is characterized by a high level of potential corresponding to locally uniform areas of one of the colors, an intermediate level of potential corresponding to locally uniform areas of the second color, and a low level of potential corresponding with locally uniform areas of the background.

There are two steps in the development of the image in this process: (1) particles of one color are attracted to areas of the electrostatic latent image of high potential and (2) particles of a second color are attracted to areas of low potential. It should be noted that this process depends in practice on the provision of different inks in separate baths so as to develop in separate steps two different areas of the electrostatic latent image.

U.S. Pat. No. 4,264,185 (Ohta) describes a process in which areas of an electrostatic latent image corresponding to two colors in an original document are developed. Ohta's process applies toners of different colors and polarities to the latent image, using separate mechanisms. In order to repel other, undesired toner particles from one development unit, a bias voltage of opposite polarity is applied to the latter unit, and vice-versa.

Ohta's process may use separate baths of the two toners, or a single partitioned bath with liquid communication between the compartments. Even where a single partitioned bath is used, the latent image is developed in two distinct steps. It is unclear from the disclosure in this patent how the question of clean-up of the background is to be dealt with, if at all.

In U.S. Pat. No. 4,562,129 (Tanaka), there is described a method of forming monochromatic or dichromatic copy images by use of a developer comprising a high-resistivity magnetic carrier and a nonmagnetic insulating toner which are triboelectrically chargeable, with the result that the toner and carrier adhere to first and second image portions, respectively, of the electro-

static latent image which has at least three levels of potential.

- In "Experimental Example 1" of Tanaka, a toner of 14 microns mean particle size and resistivity of at least 10<sup>5</sup> ohmcm, triboelectrically chargeable to positive polarity, comprised styrene-acrylic copolymer (100) and red colored charge controlling pigment (5); while a carrier of 20 microns mean particle size, resistivity of 10-ohm-cm, triboelectrically chargeable to negative polarity, comprised styrene-acrylic copolymer (100), magnetic fine powder (200), carbon black (4) and silica fluidity agent (1.5); parts indicated in parentheses are by weight. The developer comprised a 1:9 mixture of toner and carrier.
- 15 The disclosures of U.S. Pat. Nos. 4,068,938, 4,264,185 and 4,562,129 are incorporated by reference herein.
- U.S. Pat. No. 4,411,976 describes a method of increasing the density of liquid developed gap transferred electrophotographic images and developing composition for use therein wherein the carrier sheet is heated either before or after transfer to a temperature less than 100 degrees C at which the binder or polymer forming the toner particles will solvate in the liquid entrained in the transferred image to increase the density of the image.
- Reference is now made to the following published patent applications and issued patents in the field of electrophotography: OB Published Patent Applications Nos. 2,169,416A and 2,176,904A and U.S. issued Patents Nos. 3,990,696, 4,233,381, 4,253,656, 4,256,820, 4,269,504, 4,278,884, 4,286,039, 4,302,093, 4,326,644, 4,326,792, 4,334,762, 4,350,333, 4,355,883, 4,362,297, 4,364,460, 4,364,657, 4,364,661, 4,368,881, 4,378,422, 4,392,742, 4,396,187, 4,400,079, 4,411,976, 4,412,383, 4,413,048, 4,418,903, 4,420,244, 4,435,068, 4,439,035, 4,454,215, 4,460,667, 4,473,865, 4,480,825, 4,501,486, 4,522,484, 4,531,824, 4,538,899, 4,582,774, 4,585,329, 4,586,810, 4,589,761, 4,598,992, 4,603,766, 4,620,699, 4,627,705, 4,678,317, the disclosures of which are incorporated by reference herein.

## SUMMARY OF THE INVENTION

It is a principal object of the present invention to provide improved dual color imaging wherein undesired uncolored areas between different colors are sought to be eliminated.

A further object of the invention is to provide for such elimination in relation to an electrostatic imaging system utilizing simultaneous development of an electrostatic latent image in two colors with a single liquid toner composition. Such a system avoids not only the drawbacks which are inherent in a similar system using a solid particulate developer, and in any color developing system requiring more than one pass and thus accurate registration of successive images, but also the possible disadvantages (especially color continuation) of a system in which separate colors are applied successively in a single pass, since as will appear hereinafter, the different colors are already mixed in a single toner liquid, so that the problem of contamination is obviated.

Commonly assigned copending U.S. Patent Applications, all of which were filed June 6, 1988, describe a dual color imaging system employing a single toner liquid and relate to particular individual aspects of the imaging system. These applications are identified by Ser. Nos. 202,322, 202,514, 202,569, 202,677, 202,688, 202,687 and 202,551.

In operating color imaging systems of the type described in U.S. Patent Applications Ser. Nos. 202,322,

202,514, 202,569, 202,677, 202,688, 202,687 and 202,551, it is found that there is in practice a tendency for undesired, relatively uncolored areas to be formed between the colors in an image due to background cleaning and removal of pigment particles at intermediate potential ranges.

It is an object of the present invention to eliminate insofar as possible such undesired relatively uncolored areas.

Other objects of the invention will become apparent from the following description.

According to a preferred embodiment of the invention, there is provided a dual color imaging process which includes the steps of forming an image having adjacent first and second areas respectively containing first and second types of pigmented particles, undesirably separated by third areas relatively free of particles of the first and second types and causing the image to flow into the third areas, thereby at least partially eliminating the third areas.

Also in accordance with an embodiment of the invention there is provided an imaging system including apparatus for forming an image having adjacent first and second areas respectively containing first and second types of pigmented particles, undesirably separated by third areas relatively free of particles of the first and second types and apparatus for causing the image to flow into the third areas, thereby to at least partly eliminate the third areas.

Treatment of a developed image in accordance with the present invention has been found to have particular utility in relation to the imaging system which is the subject of the commonly assigned copending U.S. Applications referenced above.

#### BRIEF DESCRIPTION OF THE DRAWINGS

The present invention will be more fully understood and appreciated from the following detailed description, taken in conjunction with the drawings, in which:

FIG. 1 is a schematic sectional illustration of apparatus useful in carrying out the process of the invention;

FIGS. 2A to 2D illustrate, in schematic fashion, various steps of dichromatic electrostatic imaging according to an embodiment of the invention;

FIG. 3 is an enlarged schematic sectional illustration of apparatus shown in FIG. 1 for cleaning the background of the developed image;

FIG. 4 is a schematic illustration of a pigmented particle replenishment system useful in association with the apparatus shown in FIG. 1;

FIG. 5 is a flow chart showing operation of microprocessor apparatus useful in the pigmented particle replenishment system shown in FIG. 4; and

FIG. 6 is a graphical illustration of the interface between two different colored areas on an image bearing surface which gives rise to the presence of undesired non-colored areas.

#### DETAILED DESCRIPTION OF THE INVENTION

Referring to FIG. 1 there is shown electrostatic imaging apparatus employing a liquid toner composition comprising two oppositely charged and differently colored pigmented particles. There is shown a metal drum 2 which carries a photoconductor surface 4 and which is mounted by disks 6 onto a shaft 8 to which the disks are secured by a key 10 so that the illustrated assembly,

which is provided in a light-proof housing (not shown) is operative to rotate a shaft 8.

Shaft 8 is driven in any appropriate manner (not shown) in the direction of arrow 9 past a corona discharge device 12, adapted to charge the surface of the photoconductor 4. The image to be reproduced is focused by a lens 14 upon the charged photoconductor. Since shaft 8 is grounded at 17 and disks 6 are conductive, the areas struck by light conduct the charge, or a image. Formation of the electrostatic latent image in this way is shown in FIG. 2A.

The developing liquid containing two different pigmented particles, as described herein, is circulated from any suitable source (not shown) through a pipe 16 into a development tray 18 from which it is drawn through a pipe 20 for recirculation. Development electrodes 22, which may be appropriately biased as known to the art, assist in toning the electrostatic latent image as it passes into contact with the developing liquid.

Referring now to FIG. 2B, charged toner particles referenced 23 and 25, suspended in the carrier liquid, travel by electrophoresis to the electrostatic latent image. If, as shown in FIG. 2B, photoconductor 4 is positively charged, e.g. if a selenium photoconductor is used, negatively charged pigmented particles 23 will travel to electrostatic latent image areas having generally the highest positive potential, here shown at 1000 V, while positively charged pigmented particles 25 will travel to the latent image areas having generally the lowest positive potential of 0 V. It is noted that the background carries a charge of typically 500 V. Some positively and negatively charged toner particles 25 and 23 respectively adhere thereto.

If the photoconductor is negatively charged, e.g. if a cadmium sulfide photoconductor is used, negatively charged pigmented particles travel to electrostatic latent image areas having generally the lowest negative potential, while positively charged pigmented particles travel to the latent image areas having generally the highest negative potential.

As shown in FIG. 1, the developed image, from which excess liquid has been removed by a background clean-up unit 30 and which contains differently pigmented areas having respectively positive and negative charges, is passed under a corona discharge device 44, which imposes, for example, a negative DC electrical discharge so as to convert image areas of positive charge to a negative charge and image areas of negative charge to a relatively greater negative charge.

With particular reference to the example shown in FIG. 2C, particles 23 now carry a greater negative charge than before and particles 25, which previously carried a positive charge, now carry a relatively small negative charge. As the entire developed image now carries a charge of single polarity, transfer of the image to a carrier sheet 100 (FIG. 1) may be effected, as described below in detail, by provision of a single corotron operative to charge the sheet to a polarity opposite to that of the developed image.

In an alternative embodiment, the negative DC electrical discharge may be combined with AC electrical discharge so as to narrow (or if desired to reduce to zero) the difference in surface potentials between the differently pigmented areas.

As shown in FIG. 1, a pair of register rollers 32 and 34 is adapted to feed a carrier sheet 100, which is to receive the developed image, to a transfer station, where, as shown particularly in FIG. 2D, a corona

discharge device 46 is operative to impress upon the rear of the carrier sheet a charge of polarity opposite to that of the toner particles forming the image after electrical treatment of the image by corona discharge device 44. The developed image is thus drawn towards the carrier sheet by electrophoresis. Rollers 32 and 34 are mounted onto and secured for rotation with respective axles 36 and 38.

A pick-off member 48 assists in the removal of the carrier sheet bearing the developed image from the photoconductor. The image is then fixed onto carrier sheet 100 prior to delivery to an exit tray.

A cleaning roller 56, formed of any synthetic resin known to the art and appropriate for this purpose, is driven in a direction of rotation opposite to that of the photoconductor, to scrub clean the surface thereof. To assist in this action, insulating, nonpolar liquid may be fed through a pipe 58 to the surface of the cleaning roller 56. A wiper blade 60 completes the cleaning of the photoconductive surface. Any residual charge left on the photoconductive drum is neutralized by flooding the photoconductor surface with light from a lamp 62.

As shown in FIG. 3, a background clean-up unit, referenced generally 30, comprises, according to the illustrated embodiment, a pair of rollers 74 and 76 which are rotated (by means not shown) on axles 78 and 80 respectively, in the indicated direction, counter to that of photoconductor surface 4 (arrow 9). Background clean-up unit 30 is also operative to remove excess liquid from the photoconductive surface 4, by virtue of the reverse rotation of roller 74 as indicated in FIG. 3. The use of a reverse rotating roller for removal of excess liquid is described in U.S. Pat. No. 3,907,423, the disclosure of which is incorporated herein by reference.

By way of example, it will be supposed that the image includes areas of negative black toner particles developed at 1000 volts positive potential, and areas of positive red toner particles developed at zero potential and background areas having potential at 500 volts to which some red and black toner particles adhere.

Roller 74 is charged with a positive potential of, for example, 600 volts and thus attracts black particles from the background without detaching of red toner particles from the image. Roller 76, however, is charged with a positive potential of, for example, 400 volts and thus attracts red particles from the background without detaching black toner particles from the image. Rollers 74 and 76 are provided with respective wiper blades 82 and 84 for removal and transfer of adherent pigmented particles to circulating insulating, nonpolar liquid which may be fed into the clean-up unit through a pipe 70 and out through a pipe 72.

According to an alternative embodiment, as the liquid passes through pipe 72 in the shown direction, pigmented particles suspended in the liquid are removed by a filter 31, which may be any type of conventional filtering apparatus suited for this purpose. The filtered liquid may subsequently be recirculated into clean-up unit 30 via pipe 70. It is appreciated that due to the efficient cleaning activity of rollers 74 and 76 in the region therebetween and between photoconductor surface 4, it is possible to feed unfiltered liquid toner through pipe 70.

It is to be expected in practice that some black particles will be repelled from roller 76 towards the photoconductor surface 4. Such particles are removed therefrom together with other black particles on the background areas by the operation of roller 74.

Rollers 74 and 76 are spaced about 50 to 200 microns apart, so that red particles repelled by roller 74 are attracted to roller 76 and black particles repelled by roller 76 are attracted to roller 74.

The operation of rollers 74 and 76 in the structure of FIG. 3 described above is operative to remove from the photoconductor surface particles from regions having voltages between 400 and 600 volts. Rollers 74 and 76 will remove these particles from the background region which were meant to be color free as described above as well as from regions of transition between colors as described below.

Referring now to FIG. 6, it is noted that for two adjacent colored areas the transition of photoconductor voltages is not entirely sharp, as illustrated at A. but instead is more correctly represented by a curve B. Thus there are defined at the transitions between areas of black and red color, regions at which the voltage is between 400 and 600 volts. The width of these regions is indicated by D. At these regions, the operation of the background removal apparatus is effective to remove both the red and black toner particles thus producing third, undesired uncolored areas in these regions.

Notwithstanding that the width D is relatively small, due to the fact that the undesired uncolored areas occur at a color transition, they are noticed by the human eye.

The insulating, nonpolar liquid used as the medium for toner particles as well as for other optional purposes as described herein, preferably has a resistivity in excess of about  $10^9$  ohm-cm and a dielectric constant below about 3.0. Suitable such liquids are hydrocarbons, preferably aliphatic and more preferably isomerized aliphatic hydrocarbons, as, for example, those marketed by Exxon Corporation under such trade marks as ISO-35 PAR-G, ISOPAR-H, ISOPAR-L and ISOPAR-M. which meet the preferred resistivity and dielectric requirements. Polymers useful as binders for the pigmented particles may be thermoplastic. The presently preferred polymers are known under the trade mark 35 ELVAX II, manufactured by E.I. Du Pont de Nemours & Company. The ELVAX II family are ethylene copolymers combining carboxylic acid functionality, high molecular weight and thermal stability.

The presently preferred ELVAX II resins are those designated 5720 and 5610. Other polymers which may be used are the ELVAX polymers and the ethylene/ethyl acrylate series made by Union Carbide such as those designated DPD 6169, DPDA 6182 Natural and DTDA 9169 Natural. Still other useful polymers 50 made by Union Carbide are those designated DQDA 6479 Natural 7 and DQDA 6832 Natural 7; these are ethylene/vinyl acetate resins.

The polymers are pigmented so as to render the latent image visible in two colors. The pigments may be present generally in an amount of 1-60% by weight with respect to the weight of the polymer. The selection of two pigments from the examples listed in the description which follows and/or from those otherwise known in the art may be readily performed by a person of ordinary skill in the art.

As has been set out above, two colors may be developed simultaneously by use of a toner liquid composition which comprises an insulating, nonpolar liquid having admixed therewith two different pigmented particles carrying opposite charges. It should be emphasized that the choice of colors of the pigmented particles is entirely at the discretion of the person operating the process, subject only to the condition that the pig-

mented particles should be adapted to be oppositely charged in the same medium.

Illustrative examples of potentially suitable pigments are Cabot Mogul L (black), Monastral Blue G (C.I. Pigment Blue 15 C.I. No. 74160), Quindo Magenta (Pigment Red 122), Indo Brilliant Scarlet Toner (Pigment Red 123, C.I. No. 71145), Dalamar Yellow (Pigment Yellow 74, C.I. No. 11741), blue pigment BT-383D (DuPont), yellow pigment YT-717D (DuPont), red pigment RT-455D (DuPont) and blue pigment Heli- 10 oecht Blue G0 (Bayer).

One of the two pigments may be, if desired, a finely ground ferromagnetic material, e.g. Mapico Black. Other suitable materials are metals, including iron, cobalt and nickel; various magnetic oxides including 15  $Fe_2O_3$  and  $Fe_3O_4$ ; and others known in the art. Mixtures of known magnetic materials may also be used.

In general, the liquid toner composition employed may be prepared by a method which comprises the steps of: separately wet-grinding two pigments, which 20 are respectively adapted to acquire charges of opposite polarities, preferably together with a thermoplastic polymeric binder for the pigments, in an inert medium until homogeneous and until the dispersed solids have predetermined characteristics selected from the group 25 consisting of a desired particle size range and a fibrous structure; and polarizing the pigmented particles in the resultant wet-ground composition, whereby the pigmented particles acquire charges of opposite polarities, respectively.

The polarizing step is preferably carried out by addition of either one or two charge directors to the wet-ground composition, as otherwise described herein.

More particularly, the liquid toner composition may be prepared (e.g.) by initially mixing a suitable polymer 35 together with a plasticizer and separately with each of the two selected pigments, until homogeneity is achieved. Thereafter, the mixture is allowed to cool while mixing is continued. The mixing temperature may range from about 65° to about 100° C., preferably about 90° C. Mixing times prior to cooling, typically about 90 minutes, may range between about 10 minutes and 3 hours. Any suitable mixing or blending device may be employed, such as the Ross double planetary mixer 40 (manufactured by Charles Ross & Son of Hauppauge, 45 N.Y.).

After the mixture has been cooled, it is charged to an attritor, disk mill, sand mill, impeller attrition mill, vibroenergy mill, or the like. The liquid used during the grinding operation may be, e.g., ISOPAR-H, which is 50 present in an amount of 70-90% by weight in respect of the polymer. During the grinding, the particle size is determined, for example, by centrifugal analysis using, e.g., a Horiba Centrifugal Particle Size Analyzer, Model CAPA 500, manufactured by Horiba Instruments Inc. of Irvine, Calif.

The ground material for each pigment is then dispersed, e.g., in ISOPAR-H, and mixed with a charge director to form a working dispersion having a solids content of about 0.5 to about 3% by weight. The 60 amount of charge director is dependent on its characteristics and the requirements of the use of the particular toner in question. The working dispersions for both pigments are then combined or alternatively they may be combined prior to mixing with the charge director. 65

As mentioned above, charge directors may be used in either one of two ways, in one of which a single charge director may be used to induce opposite charges on two

different pigmented particles, respectively. The use of a single charge director in conjunction with the selection of two suitable pigmented particles may be done as e.g. is illustrated in certain of the Examples, below.

Alternatively, two charge directors are used simultaneously in the same composition, whereby there is induced a positive charge on one species of particles and a negative charge on the other species of particles. Illustration of the use of two charge directors is given in certain of the Examples below.

In view of the prior art teaching that mixing oppositely charged toner particles would render them useless for developing a dual color electrostatic latent image in a single step, it is surprising that in contrast to such prior art teaching, the embodiment just described is operable. The phenomenon that oppositely charged toner particles can exist in the same liquid toner composition is of practical utility in the present context.

Examples of charge directors which according to the prior art were regarded as inducing negative charges are, e.g., magnesium, calcium and barium petronates; aluminum stearate; metal dialkylsulfosuccinates; other metal soaps such as copper oleate; and lecithin.

Examples of charge directors which according to the prior art were regarded as inducing positive charges are, e.g., manganese naphthenate, manganese octoate, zirconium octoate and cobalt octoate.

It will be appreciated by persons skilled in the art that the mechanism of charge on pigmented particles is not fully understood. The determination of polarity and degree of charge on pigmented particles is usually determined empirically, by trial and error.

When using a toner liquid which comprises two different pigmented particles, it is evidently advantageous to monitor the amount of these pigmented particles at any particular time, in order to know the amounts of each which need to be added to bring their respective concentrations in the liquid up to the desired level.

Referring now to FIG. 4, there is shown a two pigmented particle monitoring and replenishment system. Monitoring may be effected, for example, by measuring the optical density of the toner liquid as it passes through development tray feed pipe 16 (see also FIG. 1). This may be effected by way of two LEDs (light emitting diodes) referenced 92 and 94, emitting two different wavelengths of light, and by a pair of connected light detectors, referenced 96 and 98, respectively.

The different light wavelength intensities are passed on, in digital form, to a microprocessor 90, which contains information useful in correlating the different light wavelengths' intensities with concentrations of the two pigmented particles. The information contained in the microprocessor may be compiled by means of studies on similar liquids containing known concentrations of the two pigmented particles.

By way of example, it is assumed that black and blue pigmented particles are used and that the blue pigmented particle is blue light transparent and red light absorbing. For example, detector 96 utilizing blue light may thus be used to determine the concentration of black pigmented particles, while detector 98 utilizing red light may be similarly used to determine the total concentration of the two pigmented particles; thus the concentrations of both pigmented particles in the toner liquid may be determined.

Referring additionally to FIG. 5, upon receiving input from detectors 96 and 98 as described, micro-

processor 90 is programmed to operate either or both pigmented particle pumps, respectively referenced 101 and 102, once it has determined that the concentration of either or both of the pigmented particles has fallen below a desired concentration. In this way, continuous regulation and, if necessary, replenishment, of the pigmented particles is possible.

It is also clearly advantageous to be able to monitor the amount of charge director in a given toner liquid, in order to know the amount needed for replenishment, i.e. to bring its concentration in the toner liquid up to the desired level. By way of example, this may be effected by compiling tables relating the conductivity of a toner liquid to various concentrations of the particular charge director therein and, when required, measuring the conductivity of operational toner liquid for determination of the charge director concentration by reference to the tables.

When, in accordance with a particular embodiment, there are employed two charge directors in the same toner liquid whose concentrations may not necessarily change at the same rate, it appears unlikely that conductivity measurements alone could give the necessary information as to the nature of the adjustment to be made in the concentrations. In this instance it may, therefore, be necessary to measure a different physical property, e.g. the amount (%) of absorption of light at particular wave lengths, on the clear liquid (a sample of which may be prepared, for example, electrophoretically). The obtained light absorption information should also be correlated with prepared tables. It is evident that the combination of conductivity and light absorption measurements enables determination of the amount of each charge director to be added to the liquid, and also that such measurements and determination are within the competence of a person of ordinary skill in the art.

A further indication of the depletion of charge director(s) in the toner liquid may be obtained by developing patches of each color and measuring their optical densities. Optical densities which are too high indicate depletion of charge director(s), while the contrary is indicated by optical densities which are too low. Such information could be utilized in conjunction with that obtained from conductivity measurements and also from light measurements, as applicable.

When using the dual color toner composition for development, it is necessary that the electrostatic latent image to be developed comprises areas of high, low and intermediate levels of electrostatic charge. In order to generate these three levels of charge, it will be most convenient, for example, to start with material to be copied which has a uniform gray background, besides white and black areas, such as white and black typed areas, which could be imaged by conventional optical means onto the photoconductor.

In this example, the gray will be represented in the latent image by an intermediate charge level, while the white and black areas will be represented by the two other levels of charge. In a printer, the three charge levels could be generated, for example, by modulating the power of the exposing laser beams (in a laser printer) or the amount of charge which is supplied to a latent image holding substrate (in an electrostatic or ionographic printer).

Thus, in general terms, the system described herein need not be applied to copy colors which are similar to those in a colored original. As those skilled in the art will be aware, a process including copying similar col-

ors can be made feasible by the combined use of color filters, a reading element and a printing head, with the result that the colored original will be stored and used in the form of digital information which may be utilized so as to give the desired three level latent image.

The invention will now be illustrated by the following non-limiting examples. The formulations therein were used to develop latent images from black and white Letraset originals which had either a gray or colored background. The electrostatic imaging response of the photoconductor resulted in a latent image composed of areas of approximately 1300 V (first color) and 50 V (second color) on a 600 V background. The development bias was set at about 600 V.

When using the formulations of Examples I-IV, the developed image was removed from the photoconductor surface with Scotch tape, in a Savin 870 copier. When using the formulations of Examples V-VII, the developed image was transferred to paper using an additional pre-transfer corotron with a standard Savin 870 copier configuration. In Examples I-VII no background cleaning mechanism was employed.

When using the formulation of Example VIII, the developed image was transferred to paper using an additional pretransfer corotron with a test copier configuration, and in addition a separate background cleaning station with clear liquid input, as described herein, was used. For this Example, the electrostatic imaging response of the photoconductor resulted in a latent image composed of areas of approximately 1000 Volts (first color), 50 Volts (second color) and a 500 Volt background. The development bias was set at about 600 Volts and the cleaning rollers 74 and 76 in the configuration of FIG. 3 were set at positive 600 Volts and 400 Volts respectively.

It is to be particularly noted that in accordance with the present invention, the developed image in all cases may be subjected to fusing temperatures at about 120° C. or higher on a hot plate fuser, in order to eliminate undesired relatively uncolored areas between adjacent colors. In an alternative procedure which achieves the same result, a roll fuser configuration is used with some pressure, at about 100° C.

It is noted that even though such heating eliminates some or all of the undesired relatively uncolored areas, the narrow width of such areas requires only a minimal amount of image flow and thus such image flow has an insubstantial effect on image resolution.

These temperatures relate to the use of Elvax II as binder, but in the case of other polymeric binders the appropriate temperatures necessary for elimination of the uncolored areas may be readily ascertained by one skilled in the art. Replacing part of the polymeric binder with a wax has been found to lower the temperature needed in order to achieve the objective of the invention, i.e. elimination of the uncolored areas. Suitable waxes for this purpose are, e.g., those described in the following table, in which the listed physical properties are to be regarded as approximate values:

| Wax          | m.p. (°C.) | iodine value | acid value |
|--------------|------------|--------------|------------|
| Bamboo leaf  | 80         | 8            | 14.5       |
| Caranda      | 80-84      | 8-9          | 5-10       |
| Carnauba     | 83-86      | 7-13         | 3-10       |
| Montan       | 76-86      | 14-17        | 23-31      |
| Ouricury     | 79-84      | 7-8          | 3-21       |
| Palm         | 74-86      | 9-17         | 5-11       |
| Hydrogenated | 84-88      | 2-9          | 1-5        |

-continued

| Wax            | m.p. (°C.) | iodine value | acid value |   |
|----------------|------------|--------------|------------|---|
| Castor Oil     |            |              |            |   |
| Chinese insect | 81-84      | 1.4          | 2-1.5      | 5 |
| Indian Corn    | 81         | 4.2          | 1.9        |   |
| Shellac        | 79-82      | 6-8          | 12-24      |   |

Examples I-IV and VI illustrate an embodiment of the invention in which a single charge director suffices for the two pigmented particles in the toner compositions to become oppositely charged. Examples V, VII and VIII illustrate an embodiment of the invention in which two charge directors are used to render the two pigmented particles in the toner compositions oppositely charged.

## EXAMPLE I

- (a) 1000 g. Elvax II 5720 resin (DuPont) and 500 g. Isopar L were mixed in a Ross double planetary mixer for 1 hour at 90° C., then for a further hour after addition of 250 g. Mogul L carbon black (Cabot) which had been wetted by 500 g. Isopar L, and finally for another hour after addition of 2000 g. Isopar L preheated to 110° C. Stirring was continued in absence of heating until the temperature reached 40 C. 3050 g. of the resultant mixture was milled in a Sweco M-18 vibratory mill (containing 0.5" alumina cylinders) with 4000g. Isopar L for 20 hours at 34° C.; the average particle size of the product was 2.4 microns. 30
- (b) 1200 g. Elvax II 5720 (DuPont) and 1000 g. Isopar L were mixed together in a Ross double planetary mixer at 90° C. for 1 hour; 2600 g. preheated Isopar L were then added and the mixing continued for a further 30 minutes at 100° C. The mixture was allowed to cool while continuing stirring until the temperature reached 40° C. 35
- (c) An S-0 attritor with 3/16" stainless steel balls was charged with 125 g. of the product from part (b). 2.5 g. blue pigment BT-383D (DuPont), 0.2 g. nigrosine (Solvent Black 7, Bayer) and 80 g. Isopar L. The mixture was ground for 15 hours; the final average particle size was 2.6 microns. 40
- (d) The product of part (c) was diluted to a 1.5% solids content with Isopar H, and 800 grams of it were mixed with 800 g. of the diluted product of part (a), which had already been separately diluted to a 1.5% solids content with Isopar H, and with 15 ml. of 6% Zirconium Octoate (ICN Biomedicals K+K Labs.). In this mixture, the Zirconium Octoate charge director renders the black pigmented particles negatively charged and the blue pigmented particles positively charged. 45

## EXAMPLE II

- (a) 500 g. Elvax II 5720 (DuPont) and 500 g. Isopar L were mixed together in a Ross double planetary mixer at 90° C. for 1 hour. Then 80 g. Cab-O-Sil M5 (Cabot) and 58.6 g. YT-717D yellow pigment were added and mixing was continued for 30 minutes; 1000 g. preheated Isopar L were then added and the mixing continued for 1 hour. The mixture was allowed to cool while continuing stirring until the temperature reached 40° C. 60
- (b) 535 g. of the product of part (a) and 803 g. Isopar L were ground together in a Sweco M-18/5 VM-2 vibratory mill with 0.5" alumina grinding medium for 65

250 hours; the average particle size of the product was 1.96 microns.

- (c) The product of part (b) was diluted to a 1.5% solids content with Isopar H, and 800 grams of it were mixed with 800 g. of the diluted product of part (a) of Example I, which had already been separately diluted to a 1.5% solids content with Isopar H, and with 8 ml. of 6% Zirconium Octoate (ICN Biomedicals K+K Labs.). In this mixture, the Zirconium Octoate charge director renders the black pigmented particles negatively charged and the yellow pigmented particles positively charged.

## EXAMPLE III

- (a) An S-O attritor with 3/16" stainless steel balls was charged with 100 g. of the product from part (b) of Example I, 2 g. red pigment RT-455D (DuPont), 0.2 g. nigrosine (Solvent Black 7, Bayer) and 80 g. Isopar L. The mixture was ground for 24 hours; the final average particle size was 1.6 microns.
- (b) The product of part (a) was diluted to a 1.5% solids content with Isopar H, and 750 grams of it were mixed with 750 g. of the diluted product of part (a) of Example I, which had already been separately diluted to a 1.5% solids content with Isopar H, and with 15 ml. of 6% Manganese Naphthenate (ICN Biomedicals K+K Labs.). In this mixture, the Manganese Naphthenate charge director renders the black pigmented particles negatively charged and the red pigmented particles positively charged.

## EXAMPLE IV

- (a) An S-O attritor with 3/16" stainless steel balls was charged with 100 g. of the product from part (b) of Example I, 2 g. red pigment RT-455D (DuPont), 0.2 g. Dimanane (quaternary ammonium salt, Bayer) and 80 g. Isopar L. The mixture was ground for 24 hours; the final average particle size was 1.6 microns.
- (b) The product of part (a) was diluted to a 1.5% solids content with Isopar H, and 1200 grams of it were mixed with 1200 g. of the diluted product of part (a) of Example I, which had already been separately diluted to a 1.5% solids content with Isopar H, and with 12 ml. of 6% Manganese Naphthenate (ICN Biomedicals K+K Labs.). In this mixture, the Manganese Naphthenate charge director renders the black pigmented particles negatively charged and the red pigmented particles positively charged.

## EXAMPLE V

- (a) 1000 g. Elvax II 5720 (DuPont) and 1000 g. Isopar L were mixed together in a Ross double planetary mixer at 90° C. for 1 hour. Then 60.2 g. Cab-O-Sil M5 (Cabot) and 189.75 g. RT-455 D red pigment (DuPont) were added and mixing was continued for 30 minutes; 1000 g. preheated Isopar L were then added and the mixing continued for 1 hour. The mixture was allowed to cool while continuing stirring until the temperature reached 40° C.
- (b) An S-1 attritor with 3/16" stainless steel balls was charged with 940 g. of the product from part (a) and 940 g. Isopar L. The mixture was ground for 22 hours; the final average particle size was 1.6 microns.
- (c) The product of part (b) was diluted to a 3.0% solids content with Isopar H, and 750 grams of it were mixed with 750 g. of the diluted product of part (a) of Example I, which had already been separately diluted to a 3.0% solids content with Isopar H, and with 10 ml. of 18% Zirconium Octoate (Nuxtra, Nuodex Inc.)

and 3 ml. OLOA 1200 (Oronite Division of Chevron Chemical Co.). In this mixture, both the Zirconium Octoate and the OLOA act as charge directors and render the black pigmented particles negatively charged and the red pigmented particles positively charged. While the mechanism of action of the two charge directors is at present not entirely understood, it is believed that one charge director renders the black pigmented particles negatively charged, and that the other charge director renders the red pigmented particles positively charged.

#### EXAMPLE VI

- (a) An S-O attritor with 3/16" stainless steel balls was charged with 100 g. of the product from part (b) of Example I, 2.8 g. blue pigment BT-383D (DuPont), 0.56 g. oxalic acid and 80 g. Isopar L. The mixture was ground for 21 hours; the final average particle size was 2.7 microns.
- (b) The product of part (a) was diluted to a 3.0% solids content with Isopar H, and 800 grams of it were mixed with 800 grams of the diluted product of part (a) of Example I, which had already been separately diluted to a 3.0% solids content with Isopar H, and with 10 ml. of 10% lecithin solution (Fisher Scientific Co.) in Isopar H. In this mixture, the lecithin charge director renders the black pigmented particles negatively charged and the blue pigmented particles positively charged.

#### EXAMPLE VII

- (a) 1000 g. Elvax II 5720 resin (DuPont) and 500 g. Isopar L were mixed in a Ross double planetary mixer for 1 hour at 90° C., then for a further hour after addition of 250 g. Mogul L carbon black (Cabot) which had been wetted by 500 g. Isopar L, and finally for another hour after addition of 2000 g. Isopar L preheated to 110° C. Stirring was continued in absence of heating until the temperature reached 40° C. 35 3050 g. of the resultant mixture was milled in a Sweco M-18 vibratory mill (containing 0.5" alumina cylinders) with 4000 g. Isopar L for 20 hours at 40° C.; the average particle size of the product was 2.5 microns.
- (b) An S-O attritor with 3/16" stainless steel balls was charged with 100 g. of the product from part (b) of Example I, 2.8 g. red pigment RT-455D (DuPont) and 70 g. Isopar L. The mixture was ground for 22 hours; the final average particle size was 1.6 microns.
- (c) The product of part (a) was diluted to a 3.0 % solids content with Isopar H, and 1000 grams of it were mixed with 10 ml. of 10% lecithin solution (Fisher Scientific Co.) in Isopar H.
- (d) The product of part (b) was diluted to a 3.0% solids content with Isopar H, and 1000 grams of it were mixed with 1 ml. of SN-6535 B (Philip A. Hunt Chemical Corp.).
- (e) The products of parts (c) and (d) were mixed together after 1 hour. In this mixture, the lecithin and SN-6535 B act as charge directors and render the black pigmented particles negatively charged and the red pigmented particles positively charged. While the mechanism of action of the two charge directors is at present not entirely understood, it is believed that one charge director renders the black pigmented particles negatively charged, and that the other charge director renders the red pigmented particles positively charged.

#### EXAMPLE VIII

- (a) An S-1 attritor with 3/16" stainless steel balls was charged with 1000 g. of the product from part (b) of Example I, 28 g. Heliocht Blue GO blue pigment (Bayer) and 700 g. Isopar L. The mixture was ground for 21 hours; the final average particle size was 2.1 microns.
- (b) The product of part (a) of Example VII was diluted to a 3.0% solids content with Isopar H, and 1500 grams of it were mixed with 6 ml. of 10% lecithin solution (Fisher Scientific Co.) in Isopar H.
- (c) The product of part (a) of Example VIII was diluted to a 3.0% solids content with Isopar H, and 1500 grams of it were mixed with 0.75 ml. of SN-6535 B (Philip A. Hunt Chemical Corp.).
- (d) The products of parts (b) and (c) were mixed together after 3 hours. In this mixture, the lecithin and SN-6535 B act as charge directors and render the black pigmented particles negatively charged and the blue pigmented particles positively charged. While the mechanism of action of the two charge directors is at present not entirely understood, it is believed that one charge director renders the black pigmented particles negatively charged, and that the other charge director renders the blue pigmented particles positively charged.

While the invention has been particularly described with respect to certain embodiments, it will be appreciated by the person skilled in the art that many modifications and variations may be made. The invention is therefore not to be regarded as limited to such embodiments, which are merely illustrative. Rather, the invention is defined only in accordance with the claims which follow:

We claim:

1. A dual color imaging process which comprises the following steps:  
forming an image having adjacent first and second areas respectively containing first and second types of pigmented particles and desirably uncolored background areas;  
removing unwanted pigmented particles from said background area and undesirably removing particles from the juncture of said first and second areas such that they are undesirably separated by third areas relatively free of particles of said first and second types;  
transferring the image to a final substrate; and subsequently causing said image to flow into said third areas, thereby at least partially eliminating said third areas.
2. A process according to claim 1 and wherein said step of causing comprises the step of heating said image.
3. A process according to claim 1, wherein said image is obtained by electrostatic imaging.
4. A process according to claim 1, wherein said image is produced by employing a liquid toner composition which comprises an insulating, nonpolar liquid having admixed therewith two different particulate pigments carrying opposite charges.
5. A process according to claim 2, wherein said image is produced by employing a liquid toner composition which comprises an insulating, nonpolar liquid having admixed therewith two different particulate pigments carrying opposite charges.
6. A process according to claim 5, wherein said composition also comprises at least one polymeric binder for the particulate pigments.

7. A process according to claim 6, wherein said composition also comprises at least one binder wax.

8. A process according to claim 6, wherein said at least one polymeric binder comprises an ethylene copolymer including carboxylic acid functionality.

9. A process according to claim 8, wherein said image flow is effected by a hot plate fuser and the temperature is higher than about 120° C.

10. A process according to claim 8, wherein said image flow is effected by a roll fuser with pressure and the temperature is equal to or higher than about 100° C.

11. A process according to claim 7, wherein said at least one polymeric binder comprises an ethylene copolymer including carboxylic acid functionality.

12. A process according to claim 11, wherein said image flow is effected by a hot plate fuser and the fusion temperature is lower than about 120° C.

13. A process according to claim 11, wherein said image flow is effected by a roll fuser with pressure and the temperature is lower than about 100° C.

14. A process according to claim 7, wherein said at least one binder wax is selected from the group consisting of Bamboo leaf, Caranda, Carnauba, Montan, Ouricury, Palm, Hydrogenated Castor Oil, Chinese insect, Indian Corn and Shellac waxes.

15. A process according to claim 12, wherein said at least one binder wax is selected from the group consisting of Bamboo leaf, Caranda, Carnauba, Montan, Ouricury, Palm, Hydrogenated Castor Oil, Chinese insect, Indian Corn and Shellac waxes.

16. A process according to claim 13, wherein said at least one binder wax is selected from the group consisting of Bamboo leaf, Caranda, Carnauba, Montan, Ouricury, Palm, Hydrogenated Castor Oil, Chinese insect, Indian Corn and Shellac waxes.

17. An imaging system comprising:

means for forming an image having adjacent first and second areas respectively containing first and second types of pigmented particles and desirably uncolored background areas;

means for removing unwanted pigmented particles from said background regions and also undesirably removing pigment from the juncture of said first and second areas so that they are undesirably separated by third areas relatively free of particles of said first and second types; and

means for causing flow of the image into said third areas, thereby to at least partially eliminate said third areas.

18. An imaging system according to claim 17 and wherein said means for causing comprises means for heating said image which is insufficient to cause flow of the image.

19. A system according to claim 17 and wherein said image is formed of a liquid toner composition and said means for forming comprises a development electrode biased at an electrostatic potential level intermediate the surface potential of areas on a photoconductor corresponding to said first and second areas.

20. A system according to claim 18 wherein said image is formed of a liquid toner composition and said means for forming comprises a development electrode biased at an electrostatic potential level intermediate the surface potential of areas on a photoconductor corresponding to said first and second areas.

21. A system according to claim 17, and wherein said liquid toner composition also comprises a polymeric binder for said pigmented particles.

22. A system according to claim 21, and wherein said toner composition also comprises at least one charge director.

23. A system according to claim 22 and wherein said at least one charge director is operative to induce on said first type of pigmented particles charges of a first polarity and to induce on said second type of pigmented particles charges of an opposite polarity.

24. A system according to claim 23, and wherein said at least one charge director comprises a single charge director.

25. A system according to claim 23, and wherein said at least one charge director comprises first and second charge directors, said charge directors being operative to induce on said first type of pigmented particles charges of a first polarity and to induce on said second type of pigmented particles charges of an opposite polarity.

26. A system according to claim 18, and also comprising means for removing unwanted pigmented particles from a background area of the developed image defined by said third portion.

27. A system according to claim 1, and wherein said means for removing unwanted pigmented particles comprises:

first removal means biased at a potential between (i) the average surface potential of the background area and, (ii) the potential of said first portion, for the removal of said first type of pigmented particles from the background area; and

second removal means biased at a potential between (i) the average surface potential of the background areas, and (ii) the potential of said second portion, for the removal of said second type of pigmented particles from the background area.

28. A system according to claim 26, and wherein said means for removing unwanted pigmented particles comprises:

first removal means biased at a potential between (i) the average surface potential of the background area, and (ii) the potential of said first portion, for the removal of said first type of pigmented particles from the background area; and

second removal means biased at a potential between (i) the average surface potential of the background areas, and (ii) the potential of said second portion, for the removal of said second type of pigmented particles from the background area.

29. A system according to claim 27, and wherein said first and second removal means are spaced from each other such that said second type of pigmented particles is repelled from said first removal means and is attracted thereafter to said second removal means.

30. A system according to claim 27, wherein said means for removing unwanted pigmented particles further comprises:

a liquid retaining housing associated with said first and second removal means; and

means for circulating a liquid within said housing and around said first and second removal means.

31. A system according to claim 30, and wherein said means for removing unwanted pigmented particles also comprises means for mechanically transferring removed pigmented particles to said circulating fluid.

32. A system according to claim 31 wherein said means for removing unwanted pigmented particles also comprises means for filtering pigmented particles from said circulating fluid.

33. A system according to claim 17, and also comprising means for converting the charges of said first and second types of pigmented particles from charges of opposite polarities to charges having the same polarity.

34. A system according to claim 33, and wherein said means for converting comprise means for imposing on said pigment particles an electrical discharge.

35. A system according to claim 17, and also comprising means for regulating the concentration of said first and second types of pigmented particles in said liquid toner composition.

36. A system according to claim 22, and also comprising means for regulating the concentration of said at least one charge director in said liquid toner composition.

37. A system according to claim 35, and wherein said means for regulating the concentration of said pigmented particles comprises:

means for measuring the light absorption of the liquid toner at two different wavelengths of light;

means for determining the concentrations of the first and second pigmented particles in said composition; and

means for selectively replenishing one or both of said pigmented particles in said liquid toner composition.

38. A system according to claim 37 and wherein said at least one charge director comprises first and second charge directors and said means for regulating the concentration of said at least one charge director in said liquid toner composition comprises means for separately regulating the concentrations of said first and second charge directors.

39. A system according to claim 36 and wherein said means for removing excess liquid is also operative for removing unwanted pigmented particles from the background area.

40

40. A system according to claim 19, and wherein said liquid toner composition comprises a polymeric binder for said pigmented particles.

41. A system according to claim 20, and wherein said liquid toner composition comprises at least one binder wax.

42. A system according to claim 40, wherein said at least one polymeric binder comprises an ethylene copolymer including carboxylic acid functionality.

43. A system according to claim 42, wherein said image flow is effected by a hot plate fuser and the temperature is higher than about 120° C.

44. A system according to claim 42, wherein said image flow is effected by a roll fuser with pressure and the temperature is about 100° C.

45. A system according to claim 40, wherein said at least one binder comprises an ethylene copolymer including carboxylic acid functionality.

46. A system according to claim 45, wherein said image flow is effected by a hot plate fuser and the temperature is lower than about 120° C.

47. A system according to claim 45, wherein said image flow is effected by a roll fuser with pressure and the temperature is lower than about 100° C.

48. A system according to claim 41 wherein said at least one binder wax is selected from the group consisting of Bamboo leaf, Caranda, Carnauba, Montan, Ouricury, Palm, Hydrogenated Castor Oil, Chinese insect, Indian Corn and Shellac waxes.

49. A system according to claim 45 wherein said at least one binder wax is selected from the group consisting of Bamboo leaf, Carnauba, Montan, Ouricury, Palm, Hydrogenated Castor Oil, Chinese insect, Indian Corn and Shellac waxes.

50. A system according to claim 46 wherein said at least one binder wax is selected from the group consisting of Bamboo leaf, Caranda, Carnauba, Montan, Ouricury, Palm, Hydrogenated Castor Oil, Chinese insect, Indian Corn and Shellac waxes.

\* \* \* \* \*

45

50

55

60

65